

H. A. WAGNER.

PROCESS OF SEPARATING METALS FROM ORES.

APPLICATION FILED JAN. 27, 1914.

1,115,351.

Patented Oct. 27, 1914.



Witnesses

*W. S. McLowell*  
*P. Bredkamp*

<sup>Inventor</sup>  
*Herman A. Wagner*

*By Victor J. Evans*

Attorney

# UNITED STATES PATENT OFFICE.

HERMAN A. WAGNER, OF EAST ORANGE, NEW JERSEY.

## PROCESS OF SEPARATING METALS FROM ORES.

1,115,351.

Specification of Letters Patent. Patented Oct. 27, 1914.

Application filed January 27, 1914. Serial No. 814,767.

To all whom it may concern:

Be it known that I, HERMAN A. WAGNER, a citizen of Great Britain, residing at East Orange, in the county of Essex and State of New Jersey, have invented new and useful Improvements in Processes of Separating Metals from Ores, of which the following is a specification.

The object of the present invention is the complete recovery of metals from their ores in a thoroughly economical manner.

The invention relates particularly to the recovery of such metals as copper, zinc, and the like, from sulfid and similar ores, by electrolysis in an aqueous bath comprising a solution of a soluble salt, particularly sodium chlorid, although other salts may be employed, the selection of the best salt to employ, depending largely upon the character of the particular ore under treatment.

The process is preferably carried out in an electrolytic vat provided with an active diaphragm, particularly such a diaphragm as is described and claimed in my U. S. Patent No. 1,077,444 dated Nov. 4, 1913, although other similar diaphragms may if desired be employed.

The accompanying drawing shows a suitable apparatus in which the process may be carried out, and in said drawing 1 represents a suitable tank or vat, provided with a diaphragm comprising side plates 2 and 2' of a pervious and substantially inert material, such as burnt porous clay, asbestos or the like containing a filling 3 composed of a material made from pumice stone, charcoal, and manganese dioxid, which materials in a granular condition are treated with a solution of a mercuric salt, such as mercuric chlorid, and preferably also with a hydrogen absorbing agent, such as palladium, which will preferably be used in the form of a palladium compound, such as palladium chlorid, after which the granular material is dried and treated at a temperature of 100 to 150° C., with vapor of formaldehyde or other gaseous medium capable of reducing the mercuric chlorid and palladium chlorid, but not capable of reducing the manganese dioxid at said temperature.

4 represents the anode and 5 the cathode, immersed in a bath which as above stated may consist of a solution of sodium chlorid in water.

The ore to be treated is introduced through

the chute 6, preferably in a finely ground or pulverized condition, and the electric current passing from the anode to the cathode carries the zinc or copper or other valuable metal of the ore to the cathode where it is deposited, and liberates chlorin or other suitable reagent at the anode, which being in a nascent state readily attacks the metals contained in the ore and carries the same into solution.

At 7 is shown suitable valved pipe connections for introducing salt solution, and at 8 are shown suitable valved pipe connections for withdrawing the saline solutions when it is desired to clean the cell, or at other times.

At 9 is illustrated any suitable form of stirring or agitating device which may be employed for keeping the solution in the anode compartment agitated, in order to maintain the ore either wholly or partly in suspension, and at 10 is shown a suitable man-hole closure which may be removed, to assist in removing the undecomposed ore, tailings and the like from the bottom of this compartment. If desired a coil of pipe 11 may be provided within the anode compartment, for the purpose of heating the electrolyte. If desired the agitation may also be produced by the introduction of a current of air at or near the bottom of the anode compartment.

It will be noted that a valuable feature of this invention is the use of the diaphragm described and claimed in my Patent No. 1,077,444, above referred to, by means of which hydrogen liberated in the cathode compartment is prevented from passing into the anode compartment, even if more or less of this hydrogen becomes dissolved in the liquid constituting the bath, since said hydrogen will at once be oxidized by the manganese diozid in the diaphragm. The metallic mercury increases the conductivity of the diaphragm, and acts, perhaps in the state of sodium amalgam, as an assistant to the travel of the metal ions, from the anode to the cathode. The presence of a hydrogen absorbing agent, such as the palladium black in the diaphragm by catalytic action, materially increases the rate of speed of the various chemical reactions, and apparently also the electrolysis, as does also the mercury, and moreover this palladium being a particularly active hydrogen absorbing agent, absorbs the hydrogen set free in the vicinity

of the diaphragm or within the diaphragm itself, to aid the oxidation of this hydrogen by the manganese dioxid, apparently by catalysis, and to prevent the action of this 5 hydrogen upon the chlorin evolved at the surface of the anode.

I have found by investigation that by the use of this process it is possible to extract the metals from the ores as above referred 10 to, in a very economical and complete manner, both as to the cost of labor, electric current used, and original cost of plant.

The anode 4 must obviously be made of a refractory material which is not readily attacked by chlorin and similar reagents, such 15 a material as graphilized carbon being found to be suitable. The cathode 5 may be made of any suitable material, such as the metal which is being extracted from the particular ore under treatment.

What I claim is:-

1. A process of extracting metals from their ores by electrolysis, which comprises 25 passing a current from an anode to a cathode, both being immersed in a suitable electrolyte, holding the ore in the anode compartment, the liquid in the anode compartment being kept separate from the liquid in the cathode compartment, and 30 while maintaining a depolarizing material including an oxidizing agent, in the path of the current, between said anode and said cathode.

2. A process of extracting metals from 35 their ores by electrolysis, which comprises passing a current from an anode to a cathode, both being immersed in a suitable electrolyte, holding the ore in the anode compartment, the liquid in the anode compartment being kept separate from the liquid in the cathode compartment, and 40 while maintaining a depolarizing material including an oxidizing agent and mercury, in the path of the current, between said anode and said cathode.

3. A process of extracting metals from 50 their ores by electrolysis, which comprises passing a current from an anode to a cathode, both being immersed in a suitable electrolyte, holding the ore in the anode compartment, the liquid in the anode compartment being kept separate from the

liquid in the cathode compartment, and while maintaining a depolarizing material including an oxidizing agent, mercury and 55 a hydrogen absorbing agent, in the path of the current, between said anode and said cathode.

4. A process of extracting metals from their ores by electrolysis, which comprises 60 passing a current from an anode to a cathode, both being immersed in a suitable electrolyte, holding the ore in the anode compartment, the liquid in the anode compartment being kept separate from the 65 liquid in the cathode compartment, and while maintaining a depolarizing material including a manganese dioxid, mercury, and palladium black, in the path of the current, between said anode and said cathode. 70

5. A process of extracting copper, zinc and the like, from sulfid ores containing the same, which comprises suspending said ores, in the anode compartment of an electrolytic cell containing a solution of common salt, and depolarizing the cell by oxidizing any hydrogen absorbed by the cathode liquid, before said hydrogen comes into contact with the anode liquid.

6. In an electrolytic process of extracting 80 metals from their ores, the step of supplying said ore to the electrolyte in the anode compartment, while maintaining said liquid separate from, and out of contact with the hydrogen dissolved in the liquid in the 85 cathode compartment, and oxidizing said dissolved hydrogen before the same reaches the anode compartment.

7. A process of extracting copper, zinc and the like from ores containing the same, 90 which comprises suspending the ores in the anode compartment of an electrolytic cell containing a dissolved electrolyte, and depolarizing the cell, by oxidizing any hydrogen absorbed by the cathode liquid, before 95 said hydrogen comes into contact with the anode liquid.

In testimony whereof I affix my signature in presence of two witnesses.

HERMAN A. WAGNER.

Witnesses:

JOHN E. MOATS,  
H. C. MILLS.